# EUROPEAN PATENT SPECIFICATION

(11) **EP 0 693 548 B1**
(45) Date of publication and mention of the grant of the patent: **28.11.2001**
(21) Application number: 94202726.9
(22) Date of filing: 22.09.1994
(51) Int. Cl.: C11D 1/00, C11D 1/14, C11D 1/83, C11D 3/395

(54) **A stable concentrated premix and its use for manufacturing aqueous detergent compositions**
Eine stabile konzentrierte Vormischung und ihre Verwendung zur Herstellung von wässrigen Waschmittelzusammensetzungen
Un prémélange concentré stable et son utilisation pour la fabrication des compositions détergentes aqueuses

(30) Priority: 18.07.1994 WO PCT/US94/08089
(43) Date of publication of application: 24.01.1996
(73) Proprietor: THE PROCTER & GAMBLE COMPANY, Cincinnati, Ohio 45202 (US)
(72) Inventor: Barbarino, Sergio, I-80132 Napoli (IT); Biscarini, Lamberto, I-40126 Bologna (IT); Iakovides, Panos, I-00145 Rome (IT); Pinna, Raffaele, I-00194 Rome (IT)
(74) Representative: Engisch, Gautier

(56) References cited:
- EP-A- 0 244 006
- WO-A-93/15172
- WO-A-94/10272
- DE-A- 4 025 065
- DE-A- 4 237 178
- GB-A- 1 329 086
- GB-A- 1 458 798
- US-A- 4 129 514
- US-A- 4 404 040
- US-A- 5 196 146

## Description

### Technical Field

The present invention relates to a process for manufacturing aqueous detergent compositions suitable for household applications and to a stable concentrated premix used in said process.

### Background of the Invention

Liquid detergent compositions comprising surfactants and water-insoluble materials such as perfumes, fatty acids and/or soaps are well known in the art.

Such compositions can be made by a variety of processes wherein for example the different ingredients are incorporated in said compositions at different process steps. Such processes for manufacturing aqueous detergent compositions are not fully satisfying. Indeed, a problem encountered with such fully formulated compositions is the cost of their overall sourcing, e.g. it is often needed to supply different locations with said fully formulated compositions thus having to handle and ship big volumes. Accordingly, there is a need for the development of processes for manufacturing aqueous detergent compositions sourced in the most economical way.

It is thus an object of the present invention to provide a process for manufacturing aqueous detergent compositions comprising a surfactant and water-insoluble materials, said process allowing cheaper and easier sourcing.

We have now found that this object can be met by including in a process for manufacturing an aqueous detergent composition, a step wherein a stable concentrated premix is prepared, said premix comprising most of the active ingredients of the finished detergent compositions. Indeed, in the process of the present invention a stable concentrated premix is prepared by mixing, under alkaline conditions, a surfactant comprising a hydrophobic portion and a hydrophilic portion, wherein the length chain of said hydrophobic portion is C6-C10, together with water-insoluble materials such as perfumes, soaps, fatty acids. Such a premix is then diluted to obtain the desired aqueous detergent composition. In its broadest aspect, the present invention is based on the surprising finding that a stable premix can be formulated with a high concentration of actives, including water-insoluble materials, this even without any added water, i.e. other than the water coming from the raw material used. The use of such a premix in the process of the present invention for manufacturing an aqueous detergent composition allows great flexibility in the production chain while also reducing the sourcing cost. Indeed, said premix may advantageously be manufactured in only one site of production and then shipped to the various desired sites, e.g. countries, where said premix may then be turned in the desired finished product by simple dilution. Also, according to the process of the present invention the volume to handle and ship for a given amount of active ingredients is reduced.

An advantage of the stable concentrated premix of the present invention which comprises a surfactant comprising a hydrophobic portion and a hydrophilic portion, wherein the length chain of said hydrophobic portion is C6-C10, is that said premix incorporates high amount of water-insoluble materials, this without the need of any hydrotrope or any solubilizer.

Another advantage of the stable concentrated premix of the present invention is that they have good physical stability properties, even across a wide range of temperature, e.g. from 0°C to 50°C.

GB-1329086 discloses conventional methods of making detergent compositions wherein the perfume is solubilized with the aid of a specific surface active agent, an amine oxide or long chain betaine. This patent application does not disclose a process for manufacturing aqueous detergent compositions, wherein a stable concentrated premix comprising a surfactant comprising a hydrophobic portion and a hydrophilic portion, wherein the length chain of said hydrophobic portion is C6-C10, together with water-insoluble materials is prepared.

DE-A-40 25 065 discloses concentrated compositions comprising water, an alkyl glycoside, a long chain alkyl sulphate and a short chain alkyl sulphate.

DE-A-42 37 178 discloses concentrated compositions comprising a short chain alkyl oligo alkoxylate and a long chain alkyl oligo alkoxylate.

US 5, 196, 146 discloses a concentrate for making a formulation for remoring oil and grease from a surface comprising an alkoxylated diphenyl oxide sulfonate surfactant and water.

### Summary of the Invention

The present invention encompasses a process for manufacturing an aqueous detergent composition comprising from 0.5% to 10% by weight of the total composition of a surfactant being a C₆-C₁₀ alkyl sulphate or C₆-C₁₀ alkyl sulphanate or mixtures thereof, and from 0.1% to 2% by weight of the total composition of a water-insoluble material, or mixtures thereof, said process comprising the steps of:
- preparing under alkaline conditions a stable concentrated premix having a pH greater than 10 and comprising from 0.1% to 4% by weight of the total premix of a water-insoluble material, or mixtures thereof, more than 6% by weight of the total premix of said surfactant and from 55% to 86% by weight of the total premix of water, wherein said premix is prepared by adding in warm water of a temperature of from 35°C to 45°C, said surfactant, said water-insoluble material and optionally optional ingredients while stirring;
- diluting said premix in water to obtain said detergent composition.

### Detailed Description of the Invention

The present invention encompasses a stable concentrated premix having a pH greater than 10 and comprising at least a surfactant comprising a hydrophobic portion and a hydrophilic portion, wherein the length chain of said hydrophobic portion is C6-C10, and at least a water-insoluble material. By "stable" it is to be understood herein that the concentrated premix of the present invention does not substantially separate into distinct layers, upon standing for at least 8 weeks at 25 °C. By "concentrated" it is to be understood herein that the level of water present in said premix is from 55% to 86% by weight, preferably from 60% to 85% by weight and more preferably from 65% to 80%.

As a first essential element, the premix of the present invention comprises at least a surfactant comprising a hydrophobic portion and a hydrophilic portion, wherein the length chain of said hydrophobic portion is C6-C10, or mixtures thereof. Such surfactants are able to boost the cleaning performance of any composition comprising them.

Accordingly, suitable surfactants having from 6 to 10 carbon atoms in their hydrophobic portion, for use herein are C₆-C₁₀ alkyl sulphates (C₆-C₁₀SO₄), and alkyl sulphonates (C₆-C₁₀SO₃).

All these surfactants are well known in the art. The premix according to the present invention may comprise any of the above surfactants alone, or any combination thereof, depending on the end use envisioned.

Preferred surfactants for use herein are the C6-C8 alkyl sulphates and C₆-C₈ alkyl sulphonates. Such anionic surfactants can be made by well known sulphation or sulphonation processes followed by neutralization, but said anionic surfactants are more conveniently commercially available, for instance from Rhone Poulenc under the trade name Rhodapon® OLS, or from Witco under the trade name Witconate®.

The most preferred surfactant for use herein is octyl sulphate. Suitable surfactants for use herein are preferably hypochlorite compatible. According to the present invention, the stable concentrated premix of the present invention comprises more than 6% by weight of the total premix of a surfactant as defined herein, or mixtures thereof, preferably from 6.1% to 15%, more preferably from 6.5% to 12% and most preferably from 6.5% to 10% by weight.

As a second essential element, the premix of the present invention comprises at least a water-insoluble material, or mixtures thereof. By "water-insoluble material" it is to be understood herein any component that is not miscible to water at ambient temperature, i.e. from 20°C to 25°C. In other words incorporating said given component in water at ambient temperature will result in a precipitation of said component in said medium.

Typically the premix of the present invention comprises from 0.1% to 4% by weight of the total premix of a water-insoluble material, or mixtures thereof, preferably from 0.5% to 3% by weight and more preferably from 1% to 2.5% by weight.

Suitable water-insoluble materials to be used herein include the following classes of compounds, soaps and/or fatty acids or perfumes, or colorants, or dyes or mixtures thereof.

Suitable fatty acids to be incorporated in the premix of the present invention include alkali metal salts of a C₈-C₁₈ fatty acid. Suitable fatty acids for use herein can be any C₈-C₁₈ fatty acid, preferably fully saturated, preferably a sodium, potassium or lithium salt, more preferably the sodium salt. Suitable fatty acids may be selected from caprylic acid, capric acid, lauric acid, myristic acid, palmitic acid, stearic acid and mixtures of fatty acids suitably hardened, derived from natural sources such as tallow, coconut oil, ground oil and babassu oil. Said fatty acids may be used as an additional thickening aid and as suds suppressers. Typically, the premix according to the present invention comprises from 0.5% to 4%, preferably from 1% to 3% by weight of the total premix of fatty acids.

Suitable perfumes to be incorporated in the premix of the present invention include a perfume as is as well as a perfume blend. Preferred perfumes to be used herein are bleach stable perfumes, especially when said premix is used as raw material in the process of the present invention for manufacturing an aqueous detergent composition comprising bleaches. Typically, the premix herein comprises of from 0.2% to 2% by weight of the total premix of said perfume and preferably of from 0.5% to 1%.

A further essential feature of the present invention is the alkalinity of said premix. Indeed, alkalinity plays an important role in the premix stability. Accordingly the premix of the present invention has a pH as is greater than 10, preferably greater than 11, more preferably greater than 12. This is achieved by the addition of from 0.5% to 6% by weight of the total premix of a caustic alkali or mixtures thereof and preferably of from 1.5% to 3%. Suitable caustic alkalis for use herein include sodium and/or potassium hydroxide.

The stable concentrated premix of the present invention may further comprise other ingredients such as long chain amine oxides. This, for example, in an embodiment where the premix according to the present invention may be used as a raw material in order to provide aqueous detergent compositions having particular properties, such as viscous compositions. Preferred long chain amine oxides are according to the formula R₁R₂R₃NO where R₁ is primarily a C₁₂-C₁₈ alkyl group and R₂ and R₃ are C₁ to C₃ alkyl groups and even more preferred is to use a mixture of said long chain amine oxides. Indeed, such long chain amine oxides for use herein can be Genaminox^{R} LA, Gemaminox^{R} MY-X (available from Hoechst), C₁₂-C₁₄ Aromox^{R} DMMCO-W, (AKZO), Aromox DM14D-W, (AKZO) and Aromox DM14D-W (AKZO). Suitable long chain surfactants for use herein are preferably hypochlorite compatible. Particularly suitable to be used herein is a mixture of said long chain amine oxides, more specifically a mixture of a C₁₄ chain amine oxide with a C₁₂ chain amine oxide or a C₁₆ chain amine oxide, with a ratio of said C₁₄ chain amine oxide to said C₁₂ chain amine oxide of from 0.3 to 10 and a ratio of said C₁₄ chain amine oxide to said C₁₆ chain amine oxide of from 0.2 to 4.5. The stable concentrated premix according to the present invention comprises from 0% to 12% by weight of the total premix of said long chain amine oxide, or mixtures thereof. If present said long chain amine oxide are preferably at a level of from 5% to 10% and more preferably of from 6% to 8% by weight of the total premix.

The stable concentrated premix of the present invention may further comprise other optional ingredients such as silicates, silicones, other long chain surface-active agents. This, for example in an embodiment where the premix according to the present invention may be used as a raw material in order to provide aqueous detergent compositions comprising such ingredients. Suitable long chain surface-active agents include organic surface-active agents selected from anionic, nonionic, cationic, and zwitterionic surface-active agents and mixtures thereof and preferred herein are alkyl sarcosinates, paraffin sulphonates, alkyl sulphates and alkyl ether sulphates. Highly preferred optional ingredients are C12 to C14 alkyl sulphates such as sodium dodecyl sulphate or sodium lauryl sulphate.

The stable concentrated premix of the present invention may also comprise a bleaching agent, as an optional highly preferred ingredient. Bleaching agent as mentioned herein includes hypochlorite bleaching agent and preferably an alkali metal hypochlorite. Although alkali metal hypochlorites are preferred, other hypochlorite compounds may also be used herein and can be selected from calcium and magnesium hypochlorite. Preferred alkali metal hypochlorite for use herein is sodium hypochlorite. The premix according to the present invention comprises said hypochlorite bleaching agent, such that the content of active chlorine in the composition is from 0% to 8% and preferably from 0% to 3.5%. According to the present invention the ingredients of the premix are selected so that said premix is hypochlorite compatible.

An advantage of the present invention is that said stable concentrated premix can be used as a raw material suitable to allow the formulation of fully formulated detergent compositions. Accordingly said premix constitutes up to 40% by weight of said detergent composition, preferably from 15% to 40% and more preferably from 25% to 35%.

Accordingly the present invention encompasses a process for manufacturing an aqueous detergent composition, said process comprising the step of preparing a stable concentrated premix as defined herein before. Said process further comprises a dilution step where said premix is diluted with water. The extent of dilution is at the discretion of the process operator and depends on the aqueous detergent composition desired. Indeed, the process of the present invention allows to manufacture a wide range of aqueous detergent compositions including highly concentrated compositions to non-concentrated compositions, depending on the dilution levels. The aqueous detergent composition is diluted in the process of the present invention until the aqueous detergent composition obtained herein has a concentration of surfactants having from 6 to 10 carbon atoms in their hydrophobic portion, of from 0.5% to 10% by weight of the total detergent composition, preferably of from 1% to 6% and more preferably of from 2% to 5%. Accordingly, the aqueous detergent composition obtained with the process of the present invention comprises from 0.1% to 2% by weight of the total detergent composition of water-insoluble material, or mixtures thereof, preferably from 0.5% to 2% and more preferably from 1% to 1.5%. The dilution stage is conducted at or around ambient temperature. The dilution water often has a temperature of from 15°C to 35° C.

The step of preparing the premix is conducted by simply adding in lukewarm to warm water (i.e. of from 35°C to approximately 45°C) all of the desired ingredients, i.e. surfactants as defined herein before with water-insoluble materials and the optional ingredients, e.g. silicates and/or long chain surfactants, if present, this in presence of caustic to raise the pH above 10 and while stirring. Preferred in the process of the present invention the surfactants having from 6 to 10 carbon atoms in their hydrophobic portion are added ahead of the low water solubility ingredients.

In an embodiment of the present invention where a bleaching agent is desired in the aqueous detergent compositions obtained according to the process of the present invention, said bleaching agent is preferably added as the last ingredient in said process, thereby ensuring longest possible market life for said compositions.

In another embodiment of the process of the present invention for manufacturing aqueous detergent compositions, the perfumes and/or colorants and/or dyes are preferably added during or after the dilution step, thereby ensuring great flexibility in adapting the aqueous detergent compositions to different market places. The aqueous detergent compositions obtained according to the process of the present invention may be used for a variety of cleaning purposes in any hard surfaces application including toilet bowl cleaning, in dishwashing applications, including hand dishwashing as well as washing with automatic dishwashing machines. Said compositions are suitable to be used as a pretreatment composition for treating dishes especially pans, pots kitchen grills and/or any kitchenware soiled by though food stains/encrustations.

### Examples

The following premix according to the present invention were prepared.

| Premix (% weight) | I | II | III | IV | V | VI | V |
|---|---|---|---|---|---|---|---|
| C12/14 amine oxide | / | / | / | 8 | 6 | 8 | / |
| C14 amine oxide | 6 | 5 | 4.5 | / | / | / | / |
| C16 amine oxide | 4 | 4.5 | 3 | / | 0.3 | / | / |
| octyl sulphate | 7 | 9 | 5 | 7 | 6.5 | 8 | 7.5 |
| C8/C10 amine oxide | 3 | / | 2 | / | / | / | / |
| fatty acid | 1.1 | 1.4 | 0.9 | 1 | 1.5 | 1 | 2.2 |
| sodium hydroxide | 0.6 | 2.6 | 4 | 3 | 2 | 3 | 3 |
| perfume | / | 0.8 | 0.8 | 0.7 | 0.5 | 0.7 | 0.7 |
| Silicate | 1 | 1 | 1 | / | / | / | 1 |
| Water | up to 100 | | | | | | |

According to the process of the present invention the above mentioned premix were prepared by simply mixing in warm water (about 45°C) the surfactants comprising a hydrophobic portion and a hydrophilic portion, wherein the length chain of said hydrophobic portion is C6-C10. The resulting mix was maintained at this temperature while pre-melted fatty acid was added with stirring. This was followed by addition of caustic soda and perfume under agitation. After a few minutes of stirring to ensure complete dissolution of the water-insoluble materials, the long chain surfactants (e.g. amine oxide) were added if desired. The resulting premix was allowed to stir for another 30 minutes.

All the above mentioned concentrated premix were stable.

The above mentioned premix were diluted with water to yield aqueous detergent compositions, i.e. the finished products. Indeed, the above premix were diluted with water at 1:3 ratio (three parts of water for each part of premix).

## Claims

1. A process for manufacturing an aqueous detergent composition comprising from 0.5% to 10% by weight of the total composition of a surfactant being a C₆-C₁₀ alkyl sulphate or C₆-C₁₀ alkyl sulphonate or mixtures thereof and from 0.1% to 2% by weight of the total composition of a water-insoluble material or mixtures thereof, said process comprising the steps of:
- preparing under alkaline conditions a stable concentrated premix having a pH greater than 10 and comprising from 0.1% to 4% by weight of the total premix of a water-insoluble material, or mixtures thereof, more than 6% by weight of the total premix of a surfactant being a C₆-C₁₀ alkyl sulphate or C₆-C₁₀ alkyl sulphonate or mixtures thereof, and from 55% to 86% by weight of the total premix of water wherein said premix is preparated by adding in warm water of a temperature of from 35°C to 45°C, said surfactant, said water-insoluble material, and optinally optional ingredients while strirring;
- diluting said premix with water to obtain said detergent composition.

2. A process according to claim 1 wherein said surfactant is a C6-C8 alkyl sulphate and/ or sulphonates, preferably octyl sulphate.

3. A process according to any of the preceding claims wherein said water-insoluble material includes perfumes, colorants, dyes, fatty add and/or soaps.

4. A process according to any of the preceding claims, wherein said premix comprises from 6.1% to 15% by weight of the total premix of said surfactant, or mixtures thereof, preferably from 6.5% to 12% by weight and more preferably from 6.5% to 10% by weight.

5. A process according to any of the preceding claims, wherein said premix comprises from 0.5% to 3% by weight of the total premix of said water insoluble material, or mixtures thereof and preferably from 1% to 2.5% by weight.

6. A process according to any of the preceding claims, wherein said premix has a pH as is greater than 11 and preferably greater than 12.

7. A process according to any of the preceding claims, wherein said premix further comprises optional ingredients including silicates, silicones, long chain amine oxides or other long chain surface-active agents or mixtures thereof, said long chain surface-active agents including anionic, nonionic, cationic, zwitterionic surface-active agents, or mixtures thereof.

8. A process according to claim 7, wherein said anionic surfactants are alkyl sarcosinates, paraffin sulphonates, alkyl sulphates, alkyl ether sulphates, or mixtures thereof preferably C12 to C14 alkyl sulphates and more preferably sodium dodecyl sulphate and sodium lauryl sulphate.

9. A process according to claims 7 or 8 wherein said long chain amine oxides are according to the formula R₁R₂R₃NO wherein R₂ and R₃ are independently C₁-C₃ alkyl groups and R1 is C12-C18 alkyl group.

10. A process according to any of the present claims wherein said premix further comprises a bleaching agent preferably an alkali metal hypochlorite.

11. A process according to any of the claims 1 to 9 wherein said process comprises as the last step the addition of a bleaching agent, preferably of an alkali metal hypochlorite.

## Patentansprüche

1. Verfahren zur Herstellung einer wäßrigen Detergenzzusammensetzung, welche 0,5 Gew.-% bis 10 Gew.-%, bezogen auf die Gesamtzusammensetzung, von einem grenzflächenaktiven Mittel, welches ein C₆-C₁₀-Alkylsulfat oder ein C₆-C₁₀-Alkylsulfonat oder ein Gemisch hievon ist, und 0,1 Gew.-% bis 2 Gew.-%, bezogen auf die Gesamtzusammensetzung, von einem wasserunlöslichen Material oder von Gemischen hievon umfaßt, welches Verfahren die Schritte:
- Herstellen unter alkalischen Bedingungen von einem stabilen konzentrierten Vorgemisch mit einem pH-Wert von mehr als 10 und welches 0,1 Gew.-% bis 4 Gew.-%, bezogen auf das gesamte Vorgemisch, von einem wasserunlöslichen Material oder von Gemischen hievon, mehr als 6 Gew.-%, bezogen auf das gesamte Vorgemisch, von einem grenzflächenaktiven Mittel, welches ein C₆-C₁₀-Alkylsulfat oder ein C₆-C₁₀-Alkylsulfonat oder ein Gemisch hievon ist, und 55 Gew.-% bis 86 Gew.-%, bezogen auf das gesamte Vorgemisch, an Wasser umfaßt, wobei das genannte Vorgemisch durch Zusetzen des genannten grenzflächenaktiven Mittels, des genannten wasserunlöslichen Materials und wahlweise fakultativer Bestandteile unter Rühren in warmes Wasser mit einer Temperatur von 35°C bis 45°C hergestellt wird,
- Verdünnen des genannten Vorgemisches mit Wasser, um die genannte Detergenzzusammensetzung zu erhalten,
umfaßt.

2. Verfahren nach Anspruch 1, worin das genannte grenzflächenaktive Mittel von C₆-C₈-Alkylsulfat und/oder Sulfonaten gebildet ist, vorzugsweise Octylsulfat ist.

3. Verfahren nach einem der vorstehenden Ansprüche, worin das genannte wasserunlösliche Material Parfums, Färbemittel, Farbstoffe, Fettsäuren und/oder Seifen umfaßt.

4. Verfahren nach einem der vorstehenden Ansprüche, worin das genannte Vorgemisch 6,1 Gew.-% bis 15 Gew.-%, bezogen auf das gesamte Vorgemisch, von dem genannten grenzflächenaktiven Mittel oder von Gemischen hievon, vorzugsweise 6,5 Gew.-% bis 12 Gew.-% und stärker bevorzugt 6,5 Gew.-% bis 10 Gew.-% umfaßt.

5. Verfahren nach einem der vorstehenden Ansprüche, worin das genannte Vorgemisch 0,5 Gew.-% bis 3 Gew.-%, bezogen auf das gesamte Vorgemisch, von dem genannten wasserunlöslichen Material oder von Gemischen hievon und vorzugsweise 1 Gew.-% bis 2,5 Gew.-% umfaßt.

6. Verfahren nach einem der vorstehenden Ansprüche, worin das genannte Vorgemisch einen pH-Wert von mehr als 11 und vorzugsweise von mehr als 12 besitzt.

7. Verfahren nach einem der vorstehenden Ansprüche, worin das genannte Vorgemisch ferner fakultative Bestandteile einschließlich Silikaten, Silikonen, langkettigen Aminoxiden oder anderen langkettigen grenzflächenaktiven Mitteln oder Gemischen hievon umfaßt, welche genannten grenzflächenaktiven Mittel anionische, nichtionische, kationische, zwitterionische grenzflächenaktive Mittel oder Gemische hievon umfassen.

8. Verfahren nach Anspruch 7, worin die genannten anionischen grenzflächenaktiven Mittel Alkylsarcosinate, Paraffinsulfonate, Alkylsulfate, Alkylethersulfate oder Gemische hievon, vorzugsweise C₁₂-C₁₄-Alkylsulfate und stärker bevorzugt Natriumdodecylsulfat und Natriumlaurylsulfat sind.

9. Verfahren nach den Ansprüchen 7 oder 8, worin die genannten langkettigen Aminoxide der Formel R₁R₂R₃NO entsprechen, worin R₂ und R₃ unabhängig voneinander C₁-C₃-Alkylgruppen sind und R₁ eine C₁₂-C₁₈-Alkylgruppe darstellt.

10. Verfahren nach einem der vorstehenden Ansprüche, worin das genannte Vorgemisch ferner ein Bleichmittel, vorzugsweise ein Alkalimetallhypochlorit umfaßt.

11. Verfahren nach einem der Ansprüche 1 bis 9, wobei das genannte Verfahren als letzten Schritt die Zugabe eines Bleichmittels, vorzugsweise eines Alkalimetallhypochlorits umfaßt.

## Revendications

1. Procédé de fabrication d'une composition détergente aqueuse comprenant 0,5% à 10% en poids de la composition totale d'un tensioactif qui est un alkylsulfate en C₆-C₁₀ ou un alkylsulfonate en C₆-C₁₀ ou leurs mélanges et 0,1% à 2% en poids de la composition totale d'un matériau insoluble dans l'eau ou de ses mélanges, ledit procédé comprenant les étapes consistant à :
- préparer dans des conditions alcalines un pré-mélange concentré stable ayant un pH supérieur à 10 et comprenant 0,1% à 4% en poids du pré-mélange total d'un matériau insoluble dans l'eau, ou de ses mélanges, plus de 6% en poids du pré-mélange total d'un tensioactif qui est un alkylsulfate en C₆-C₁₀ ou un alkylsulfonate en C₆-C₁₀ ou leurs mélanges, et 55% à 86% en poids du pré-mélange total d'eau, ledit pré-mélange étant préparé en ajoutant dans l'eau chaude ayant une température de 35°C à 45°C, en agitant, ledit tensioactif, ledit matériau insoluble dans l'eau et en option des ingrédients optionnels ;
- diluer ledit pré-mélange avec de l'eau pour obtenir ladite composition détergente.

2. Procédé selon la revendication 1, dans lequel ledit tensioactif est un alkylsulfate et/ou alkylsulfonate en C₆-C₈, de préférence un octylsulfate.

3. Procédé selon l'une quelconque des revendications précédentes, dans lequel ledit matériau insoluble dans l'eau comprend des parfums, des colorants, des teintures, des acides gras et/ou des savons.

4. Procédé selon l'une quelconque des revendications précédentes, dans lequel ledit pré-mélange comprend 6,1% à 15% en poids du pré-mélange total dudit tensioactif, ou ses mélanges, de préférence 6,5% à 12% en poids et mieux encore 6,5% à 10% en poids.

5. Procédé selon l'une quelconque des revendications précédentes, dans lequel ledit pré-mélange comprend 0,5% à 3% en poids du pré-mélange total dudit matériau insoluble dans l'eau, ou ses mélanges et de préférence 1% à 2,5% en poids.

6. Procédé selon l'une quelconque des revendications précédentes, dans lequel ledit pré-mélange a un pH supérieur à 11 et de préférence supérieur à 12.

7. Procédé selon l'une quelconque des revendications précédentes, dans lequel ledit pré-mélange comprend en outre des ingrédients optionnels comprenant des silicates, des silicones, des oxydes d'amines à chaîne longue ou d'autres agents tensioactifs à chaîne longue ou leurs mélanges, lesdits agents tensioactifs à chaîne longue comprenant des agents tensioactifs anioniques, non ioniques, cationiques, zwittérioniques, ou leurs mélanges.

8. Procédé selon la revendication 7, dans lequel lesdits tensioactifs anioniques sont des alkylsarcosinates, des paraffinesulfonates, des alkylsulfates, des alkyléthersulfates, ou leurs mélanges, de préférence des alkylsulfates en C₁₂ à C₁₄ et mieux encore le dodécylsulfate de sodium et le laurylsulfate de sodium.

9. Procédé selon les revendications 7 ou 8, dans lequel lesdits oxydes d'amines à chaîne longue sont selon la formule R₁R₂R₃NO dans laquelle R₂ et R₃ sont indépendamment des groupes alkyle en C₁-C₃ et R₁ est un groupe alkyle en C₁₂-C₁₈.

10. Procédé selon l'une quelconque des revendications précédentes, dans lequel ledit pré-mélange comprend en outre un agent de blanchiment, de préférence un hypochlorite de métal alcalin.

11. Procédé selon l'une quelconque des revendications 1 à 9, dans lequel ledit procédé comprend comme dernière étape l'addition d'un agent de blanchiment, de préférence un hypochlorite de métal alcalin.
